

United States Patent [19]  
Park

[11] 3,919,097  
[45] Nov. 11, 1975

- [54] **LUBRICANT COMPOSITION**  
[75] Inventor: **Kisoon Park**, Charleston, W. Va.  
[73] Assignee: **Union Carbide Corporation**, New York, N.Y.  
[22] Filed: **Sept. 6, 1974**  
[21] Appl. No.: **503,686**  
[52] U.S. Cl. .... **252/48.6**; 252/8.9; 252/49.6;  
252/52 R; 252/52 A  
[51] Int. Cl. .... **C10M 1/38**; C10M 3/32;  
C10M 5/28; C10M 7/36  
[58] **Field of Search**..... 252/48.6, 49.6, 52 R, 52 A,  
252/8.9
- [56] **References Cited**  
UNITED STATES PATENTS  
3,629,310 12/1971 Bailey et al. .... 252/49.6

3,657,309 4/1972 Dexter et al. .... 252/48.6  
3,671,433 6/1972 Brenner .... 252/49.6  
3,832,328 8/1974 Eggensperger et al. .... 252/48.6

*Primary Examiner*—Delbert E. Gantz  
*Assistant Examiner*—I. Vaughn  
*Attorney, Agent, or Firm*—F. M. Fazio

[57] **ABSTRACT**

A lubricant for polyolefin carpet backing containing a copoly(oxyethylene-oxypropylene) glycol or mono-ether, a hindered phenol stabilizer, a coupling agent, a bulk wetting agent and, optionally, a corrosion inhibitor suitable for use in carpets having a polyolefin backing. The lubricant composition of this invention prevents degradation of the carpet backing while at the same time, affording good lubricity during the carpet manufacturing process.

**12 Claims, No Drawings**

## LUBRICANT COMPOSITION

## BACKGROUND OF THE INVENTION

During the past decade, polyolefins have been used extensively as backing material in the production of carpets. Normally, the polyolefinic carpet backing is lubricated to minimize shattering of the backing fibers or ribbons and to reduce wear on the tufting needles. The lubricant also prevents excessive heat build up on the needles which can cause fusion of the fiber polymer. The water soluble copoly(oxyethyleneoxypropylene) derivatives have been found effective for this use since they do not readily penetrate into the polyolefin as do lubricants such as mineral oil or the fatty acids or esters thereof. The advantages of the copoly(oxyethylene-oxypropylene) derivatives are their exceptionally good tufting lubricity and their water solubility since it is preferred to apply the lubricant to the backing from an aqueous bath. However, one of the great disadvantages of the use of these materials has been their tendency to degrade the strength properties of the polyolefin backing during heat aging of the carpet.

## SUMMARY OF THE INVENTION

The instant invention pertains to a lubricant composition for polyolefin carpet backings, such as polypropylene, having desirable thermal stability and lubricity that does not cause degradation of the polyolefin backing. This lubricant composition contains a major amount of a random or block copoly(oxyethylene-oxypropylene) glycol or monoether and minor amounts of a hindered phenol stabilizer, a coupling agent, a wetting agent and, optionally, a corrosion inhibitor, as hereinafter defined.

## DESCRIPTION OF THE INVENTION

In the production of carpets, whether with synthetic or natural fibers, a carpet backing is employed which can be either woven, spun bonded or needle punched. During the manufacture process heat build up can become a problem and it is therefore necessary to use some form of lubrication to minimize the problem. This invention pertains to a specifically defined lubricant composition suitable for use in carpet manufacturing process in which the carpet backing is a polyolefin material, such as, polypropylene or blends thereof with other polyolefins or copolymers of polypropylene. The polypropylenes find particular favor in the industry because of the desirable properties of fibers, films, ribbons, etc., thereof. These materials are all well known in the art and those skilled in the manufacture of carpets are fully familiar with the wide variety of polypropylene carpet backings that can be used. The lubricant compositions of this invention can be used in any carpet manufacturing process employing any of the suitable polypropylene carpet backings. In this application, the term polypropylene carpet backing is intended to mean those backings containing polypropylene alone, blends thereof or copolymers thereof.

When using the lubricant compositions of this invention they are employed in the conventional manner by applying them to the backing using any of the known procedures. The manner in which the lubricant is applied to the backing is of no critical importance.

The block or random copoly(oxyethylene-oxypropylene) glycol or monoether thereof which makes up a

major amount of the lubricant composition is represented by the structural formula



Wherein  $R'''$  is hydrogen or alkyl of from 1 to 12 carbon atoms, preferably 2 to 8 carbon atoms;  $q$  and  $r$  are integers, such that  $q$  comprises from 25 to 75 weight percent, preferably 35 to 65 weight percent, of the sum of  $q$  and  $r$ , and wherein said glycol or monoether has a number average molecular weight of from 500 to 30,000, preferably from 1000 to 5000. The concentration of this component in the lubricant composition should be above about 60 weight percent. An amount of from about 60 to 98 weight percent can be used, preferably from about 60 to about 94 weight percent and most preferably, from about 70 to 80 weight percent. These copoly(oxyethylene-oxypropylene) glycols and monoethers are well known and many of them are commercially available. Illustrative thereof are the copoly(oxyethylene-oxypropylene) glycols having average molecular weights of 750, 1,000, 2,200, 2,400, 3,300, 3,800, 4,000, 4,400 or 5,500 and the methyl, propyl, butyl, hexyl, 2-ethylhexyl, decyl and dodecyl monoethers thereof wherein the oxyethylene content therein can be 30, 38, 42, 50, 56, 64, 70 or 75 mole percent.

25 30 35 40 45 50 55 60 65 70 75 80 85 90 95 100

The hindered phenol stabilizers are present in the lubricant composition at a concentration of from about 0.1 to about 5 weight percent, preferably from about 0.2 to about 2 weight percent. These stabilizers are those represented by the structural formula



wherein  $R$  is (i) an alkyl group of from 1 to about 6 carbon atoms, preferably 4 to 6 carbon atoms, and most preferably the tertiary butyl group when  $X$  is either  $-COOR'$  or



or (ii) a hydrogen atom or an alkyl group of from 1 to about 6 carbon atoms, preferably 4 to 6 carbon atoms when  $X$  is



$R'$  is alkyl of from about 6 to about 22 carbon atoms; preferably 12 to 18 carbon atoms and  $n$  and  $m$  are integers of from 2 to 4, preferably 2 or 3. Many of these hindered phenols are known and illustrative thereof one can mention, octadecyl beta-(3,5-di-t-butyl-4-

hydroxyphenyl)propionate, bis[2-(3,5-di-t-butyl-4-hydroxyphenethyl)carbonyloxyethyl]sulfide and 1,1,3-triphenylolpropane.

It was found that only those hindered phenols defined by the above formula yield lubricant compositions which do not discolor the lubricant or the carpet backing on standing or on heat aging. Thus, for example, other hindered phenols such as 2,6-di-t-butyl-4-methylphenol, 2,6-di-t-butylphenol, phenyl alpha-naphthylamine, 2,2'-methylenebis-(4-methyl-6-t-butylphenol), 2,4-bis(4-hydroxy-3,5-di-t-butylphenoxy)-6-(n-octylthio)-1,3,5-triazine and 1,3,5-trimethyl-2,4,6-tris(3,5-di-t-butylhydroxybenzyl)phenol, were found unsatisfactory and we were unable to produce thermally stable carpet backing lubricants with these materials.

The lubricant composition contains a coupling agent to dissolve the hindered phenol stabilizer in both the copoly(oxyethylene-oxypropylene) glycol or mono-ether and the water with which it is diluted. This coupling agent is present in the lubricant composition at a concentration of from about 2 to about 35 weight percent, preferably from about 5 to about 30 weight percent. The suitable coupling agents are those represented by the structural formula  $R''O(CH_2CH_2O)_pH$ , wherein  $R''$  is alkyl of from about 8 to 22 carbon atoms, preferably from 11 to 18 carbon atoms, phenyl or alkylphenyl wherein the alkyl group thereof has from 1 to about 18 carbon atoms, preferably from about 6 to 12 carbon atoms, and  $p$  is an integer having the value of from about 3 to about 40, preferably from 7 to 20. These compounds are well known and commercially available; they are the adducts of from about 9 to about 15 moles of ethylene oxide with  $C_{10}$  to  $C_{20}$  linear aliphatic alcohols or alkyl phenols such as octylphenol. Illustrative of commercial products are TERGITOL Nonionic 15-S-9, or Nonionic NPX, Igepal CA-630 or RC-630 and Triton X-100.

The lubricating composition also contains from about 0.05 to about 2.5 weight percent, preferably from about 0.1 to about 1 weight percent, of a bulk wetting agent which is a random copolymer of the following structure



Wherein Me is methyl,  $x$  is from about 15 to about 100, preferably from about 20 to 75,  $d$  is from 5 to 30, preferably from about 7 to 20,  $b$  is from 0 to about 50, preferably from 0 to about 30, and  $y$  is from about 2.5 to about 7.5, preferably from about 3.2 to about 5.1. These silicone alkylene oxide copolymer bulk wetting agents are known commercially available materials and require no further description to enable one skilled in the art to fully understand which compounds are intended.

The presence of a corrosion inhibitor is not critical to this invention and it is used solely to prevent corrosion of machine parts. When present it can be present at a concentration up to about 10 weight percent, preferably from about 0.5 to 5 weight percent. Any of the known corrosion inhibitors that are miscible with the lubricant composition and used in the textile art can be used and illustrative thereof one can mention, tricresyl phosphite, triisopropanolamine, tetrapropenylsuccinic anhydride, sodium benzoate, the phosphate inhibitors, and the like.

The lubricant compositions of this invention are produced by mixing the components by conventional mixing procedures. The manner of mixing is not critical. Normally, these compositions are diluted with water before they are applied to the fabric. The concentration thereof in the aqueous mixture can vary from about 5 to 30 weight percent, preferably from about 10 to 20 weight percent. The lubricant composition is applied to the fabric or carpet backing by any conventional means such as padding, dipping, roller coating, spraying or any other suitable procedure generally employed. After it has been applied to the carpet backing at a lubricant loading of from about 2 to 5 weight percent, the carpet is manufactured by conventional tufting or other procedure. The lubricant compositions of this invention were evaluated for their thermal stability and the inertness or prevention of degradation of carpet backing by padding woven polypropylene backing with a 20 weight percent aqueous mixture of the lubricant to obtain a 4 to 5 weight percent lubricant loading on the backing. The backing was then heat set in an oven at 350°F. for two minutes and six inch (warp) by 1 inch (fill) strips were cut therefrom for evaluation. The strips were hung in an oven set at 230°F. to 258°F. with a 10 gram weight attached to the end of each strip. The heat aged samples were removed from the oven at different intervals and their tensile strengths were determined with an Instron Tensile Tester by the procedure described in ASTM D 2646.

30 The following examples further serve to illustrate the invention. Parts and percentages are by weight unless otherwise specified.

#### EXAMPLE 1

35 A lubricant composition was containing 82.7 parts of the butyl monoether of the random copoly(oxyethylene-oxypropylene) glycol having an average molecular weight of about 4400 and containing 64 mole percent oxyethylene units, 15 parts by weight of the adduct of 9 moles of ethylene oxide per mole of a  $C_{11}$  to  $C_{15}$  mixture of linear alcohols as the coupling agent, one part of stearyl beta-(3,5-di-t-butyl-4-hydroxyphenyl) propionate as the stabilizer, one part of tetrapropenylsuccinic anhydride as corrosion inhibitor and 0.3 part of



as the bulk wetting agent. An aqueous lubricant composition was prepared containing 20 weight percent of the above lubricant composition and this was padded on to polypropylene carpet backing fabric to obtain a 4 to 5 weight percent loading of the lubricant on the backing. The backing was heat set at 350°F. for 2 minutes and then the tensile strength was determined on strips by the procedure previously described.

55 For comparative purposes the same polypropylene carpet backing was coated with aqueous compositions containing the same uninhibited copoly(oxyethyleneoxypropylene) derivative (Control I), the same inhibited copoly(oxyethylene-oxypropylene) derivative containing 1 weight percent of diphenylol propane (Control II), the same copoly(oxyethylene-oxypropylene) derivative containing 1 weight percent of 2,6-di-t-butyl-4-methylphenol (Control III) and the tensile strength at break was determined. The same test was also carried out on the uncoated carpet backing (Control IV). The results of this evaluation are set forth

below after the carpet backing specimens had been heat aged at 240°F. for 116 hours and 138 hours.

|                                    | Tensile Strength at Break, lb. |           |
|------------------------------------|--------------------------------|-----------|
|                                    | 116 hours                      | 138 hours |
| Lubricant Composition of Example 1 | 78.8                           | 77.5      |
| Control I                          | less than 1                    | —         |
| Control II                         | less than 1                    | —         |
| Control III                        | less than 1                    | —         |
| Control IV                         | 80                             | 81        |

As can be seen the lubricant composition containing the defined stabilizer of this invention showed no harmful effect on the polypropylene carpet backing. Whereas all of the other lubricant compositions, Controls II and III, containing conventional stabilizers and the uninhibited lubricant (Control I) showed excessive deterioration of the backing and, in fact, complete strength loss within 24 hours of heat aging. This shows that the lubricant composition of Example 1 can be used to lubricate the polypropylene carpet backing without fear of causing any significant degradation or deterioration thereof. While Control IV showed no degradation, the non-lubricated carpet backing would present problems during the carpet manufacturing process. The results indicate that the lubricant compositions of this invention do not have a degrading effect on the polypropylene carpet backing.

#### EXAMPLE 2

A lubricant composition was prepared containing 77.7 parts of the butyl monoether of the random copoly-(oxyethylene-oxypropylene) glycol having an average molecular weight of about 4400 and containing 64 mole percent oxyethylene units, 20 parts by weight of the adduct of 9 moles of ethylene oxide per mole of a C<sub>11</sub> to C<sub>15</sub> mixture of linear alcohols, one part of bis[2-(3,5-di-t-butyl-4-hydroxy-phenethyl) carboxyloxyethyl] sulfide, one part of tetrapropenylsuccinic anhydride and 0.3 part of



An aqueous lubricant composition was prepared containing 20 weight percent of the above lubricant composition and this was padded on to polypropylene carpet backing fabric to obtain a 4 to 5 weight percent loading of the lubricant on the backing. The backing was heat set at 350°F. for 2 minutes and then the tensile strength was determined on strips by the procedure previously described.

For comparative purposes the same polypropylene carpet backing was coated with aqueous compositions containing the same uninhibited copoly(oxyethylene-oxypropylene) derivative (Control I), the same inhibited copoly(oxyethylene-oxypropylene) derivative containing 1 weight percent of 2,4,6-tris(3,5-di-t-butyl-hydroxybenzyl)phenol (Control II), the same copoly(oxyethylene-oxypropylene) derivative containing 1 weight percent of 2,4-bis(4-hydroxy-3,5-di-butyl-phenoxy)-6-(n-octylthio)-1,3,5-triazine (Control III) and the tensile strength at break was determined. The same test was also carried out on the uncoated carpet backing (Control IV). The results of this evaluation are

set forth below after the carpet backing specimens had been heat aged at 240°F. for 116 hours.

|                                    | Tensile Strength at Break, lb. |           |
|------------------------------------|--------------------------------|-----------|
|                                    | 116 hours                      | 116 hours |
| Lubricant Composition of Example 2 | 78.5                           | —         |
| Control I                          | less than 1                    | —         |
| Control II                         | less than 1                    | —         |
| Control III                        | less than 1                    | —         |
| Control IV                         | 80                             | —         |

As can be seen the lubricant composition containing the defined stabilizer of this invention showed no harmful effect on the polypropylene carpet backing. Whereas, all of the other lubricant compositions, Control I and Controls II and III, containing conventional stabilizers showed excessive deterioration of the backing and, in fact, complete strength loss within 24 hours of heat aging. This shows that the lubricant composition of Example 2 can be used to lubricate the polypropylene carpet backing without fear of causing any degradation or deterioration thereof.

#### EXAMPLE 3

A lubricant composition was prepared containing 82.7 parts of the butyl monoether of the random copoly-(oxyethylene-oxypropylene) glycol having an average molecular weight of about 4400 and containing 64 mole percent oxyethylene units, 15.0 parts by weight of the adduct of 9 moles of ethylene oxide per mole of a C<sub>11</sub> to C<sub>15</sub> mixture of linear alcohols, one part of 1,1,3-triphenylol propane, one part of tetrapropenylsuccinic anhydride and 0.3 part of the silicone wetting agent employed in Example 1. An aqueous lubricant composition was prepared containing 20 weight percent of the above lubricant composition and this was padded on to polypropylene carpet backing fabric to obtain a 4 to 5 weight percent loading of the lubricant on the backing. The backing was heat set at 350°F. for 2 minutes and then the tensile strength was determined on strips by the procedure previously described.

For comparative purposes the same polypropylene carpet backing was coated with an aqueous composition containing the same uninhibited copoly(oxyethylene-oxypropylene) derivative (Control I), and the tensile strength at break was determined. The same test was also carried out on the uncoated carpet backing (Control II). The results of this evaluation are set forth below after the carpet backing specimens had been heat aged at 250°F for 112 hours.

|                                    | Tensile Strength at Break, lb. |           |
|------------------------------------|--------------------------------|-----------|
|                                    | 112 hours                      | 112 hours |
| Lubricant Composition of Example 3 | 79                             | —         |
| Control I                          | less than 1                    | —         |
| Control II                         | 75                             | —         |

As can be seen the lubricant composition containing the defined stabilizer of this invention showed no harmful effect on the polypropylene carpet backing. Whereas, the lubricant composition of Control I showed excessive deterioration of the backing and, in fact, complete strength loss within 24 hours of heat aging. This shows that the lubricant composition of Ex-

ample 3 can be used to lubricate the polypropylene carpet backing without fear of causing any degradation or deterioration thereof.

Similar results are obtained when one uses the 2-ethylhexyl monoether or the diol in the preparation of the lubricant composition.

What is claimed is:

1. A lubricant composition comprising (A) a major amount of a random or block copoly(oxyethylene-oxypropylene) glycol or monoether thereof of the structure:



wherein  $R'''$  is hydrogen or alkyl of from 1 to 12 carbon atoms;  $q$  and  $r$  are integers such that  $q$  comprises from 25 to 75 weight percent of the sum of  $q$  plus  $r$ , and wherein said glycol or monoether has a number average molecular weight of from 500 to 30,000; (B) from 0.1 to 5 weight percent of a stabilizer of the structure:



wherein  $R$  is (i) alkyl of 1 to 6 carbon atoms when  $X$  is  $-COOR'$  or



or (ii) hydrogen or alkyl of 1 to 6 carbon atoms when  $X$  is



$R'$  is alkyl of from 6 to 22 carbon atoms;  $n$  and  $m$  are integers of from 2 to 4; (C) from 2 to 35 weight percent of a coupling agent of the structure:



wherein  $R''$  is alkyl of from 8 to 22 carbon atoms; phenyl or alkylphenyl wherein said alkyl group has from 1 to 18 carbon atoms; and  $p$  is an integer of from 3 to 40; (D) from 0.5 to 2.5 weight percent of a bulk wetting agent of the random structure:



in which  $Me$  is methyl,  $x$  is from 15 to 100,  $d$  is from 5 to 30,  $b$  is from 0 to 50, and  $y$  is from 2.5 to 7.5; and (E) from zero to 10 weight percent of a corrosion inhibitor.

5 2. A lubricant composition as claimed in claim 1 wherein (A) is present at a concentration of from about 60 to about 94 weight percent; (B) is present at a concentration of from 0.2 to 2 weight percent; (C) is present at a concentration of from 5 to 30 weight percent; (D) is present at a concentration of from 0.1 to 1 weight percent; and (E) is present at a concentration of from 0.5 to 5 weight percent.

10 3. A lubricant composition as claimed in claim 2 wherein (B) is octadecyl beta-(3,5-di-t-butyl-4-hydroxyphenyl) propionate.

4. A lubricant composition as claimed in claim 2 wherein (B) is bis[2-(3,5-di-t-butyl-4-hydroxyphenethyl) carbonyloxyethyl] sulfide.

20 5. A lubricant composition as claimed in claim 2 wherein (B) is 1,1,3-triphenylpropane.

25 6. A lubricant composition as claimed in claim 2 wherein (A) is a random copoly(oxyethylene-oxypropylene) glycol having a number average molecular weight of from 600 to 20,000.

7. A lubricant composition as claimed in claim 2 wherein (D)  $x$  is from 20 to 75,  $d$  is from 7 to 20,  $b$  is from 0 to 30 and  $y$  is from 3.2 to 5.1.

8. A lubricant composition as claimed in claim 2 wherein the bulk wetting agent (D) is:



35 9. A lubricant composition as claimed in claim 2 wherein the bulk wetting agent (D) is:



40 10. A lubricant composition as claimed in claim 3 wherein (D) is:



45 11. A lubricant composition as claimed in claim 4 wherein (D) is:



50 12. A lubricant composition as claimed in claim 5 wherein (D) is:



\* \* \* \* \*